

Dec. 23, 1958

P. M. MADER

2,865,747

PHOTOGRAPHIC COLOR DEVELOPMENT PROCESS

Filed Dec. 22, 1955

*Stage 1*



*Stage 2*



*Stage 3*



*Stage 4*



PAUL M. MADER  
INVENTOR.

*Daniel L. Mayne*  
BY  
*W.H. Jewell*  
ATTORNEY & AGENT

# United States Patent Office

2,865,747

Patented Dec. 23, 1958

1

2,865,747

## PHOTOGRAPHIC COLOR DEVELOPMENT PROCESS

Paul M. Mader, Rochester, N. Y., assignor to Eastman Kodak Company, Rochester, N. Y., a corporation of New Jersey

Application December 22, 1955, Serial No. 554,827

6 Claims. (Cl. 96—55)

This invention relates to a photographic color reproduction process involving the use of coupler compounds and color developing agents which is distinct from conventional color processes employing color development in that the dye image formation is carried out at a stage in the process at which no silver halide is present.

That is, in conventional processes of color photography employing color development, exposed silver halide emulsion layers are developed with a primary aromatic amino silver halide developing agent in the presence of a coupler compound such as the naphthol and pyrazolone coupler compounds. During the color development step the coupler compound reacts with the oxidation product of the developing agent to form a dye image in situ with the developed silver. Thereafter the silver image and residual silver halide are removed from the emulsion layer by well-known silver bleaching and fixing operations.

My process involves the use of silver halide emulsion layers containing a mixture of any of the well-known types of coupler compounds and of a non-diffusing or slowly diffusing hydroquinone derivative capable of being oxidized by the oxidized forms of high energy silver halide developers. The coupler and hydroquinone derivative are dissolved together in a low molecular weight substantially water-insoluble organic crystalloidal coupler solvent such as dibutylphthalate, and this solution is dispersed in the emulsion layer. After exposure, the emulsion layer is developed in a black-and-white developer containing as an active developing agent a substance the oxidized form of which is capable of oxidizing the hydroquinone derivative incorporated in the emulsion layer. Under these conditions, the oxidized developer formed in regions of silver development in turn oxidizes the incorporated hydroquinone derivative, giving a quinonoid image in situ with the silver image. Thereafter the emulsion layer is bleached and fixed to remove silver and residual silver halide, leaving the quinonoid image in the layer together with the coupler compound. Subsequent treatment of the layer in an alkaline solution of a color developing agent causes production of a dye image in the region of the original silver image. This dye is formed through reactions involving the color developing agent, the quinonoid substance in the image, and the coupler.

One advantageous feature of my process as compared to ordinary color development processes will be apparent. Since the bleaching and fixing operations are carried out prior to the color development step, it is possible to obtain color reproductions which have appreciably less stain in the highlight regions. In the usual color development processes, the removal of the silver and residual silver halide by bleaching and fixing solutions is carried out subsequent to color development, and any color developer remaining in the emulsion layer is usually oxidized by the bleaching solution to form undesirable stain.

The process of my invention will now be described with particular reference to the accompanying drawing.

2

## EXAMPLE

To a sample of a gelatino-bromoiode emulsion containing 0.0085 mol of silver halide was added a dispersion of the following ingredients:

|    |                                                                 |    |     |
|----|-----------------------------------------------------------------|----|-----|
| 5  | Coupler                                                         | gm | 0.5 |
|    | Sec.-octadecylhydroquinone                                      | gm | 1.5 |
|    | Dibutylphthalate                                                | cc | 3   |
|    | Gelatin (10% aqueous solution)                                  | cc | 18  |
| 10 | Sodium triisopropyl naphthalene sulfonate (5% aqueous solution) | cc | 3   |
|    | Saponin solution (0.75% aqueous)                                | cc | 14  |

The emulsion thus prepared was then coated on a film support, the resulting element appearing substantially as shown in greatly enlarged cross-sectional view in stage 1 of the drawing wherein layer 10 is the support and 11 the emulsion layer.

The sensitive element was then exposed to a suitable subject such as a color-separation image as shown in stage 1 of the drawings to record the subject in area 12 of emulsion layer 11. The exposed element was then processed as follows, all solutions being maintained at approximately 68° F.:

|    |                            |      |    |
|----|----------------------------|------|----|
| 25 | 1. Black-and-white develop | Min. | 5  |
|    | 2. Wash                    |      | 1  |
|    | 3. Harden and stop         |      | 2  |
|    | 4. Wash                    |      | 10 |
| 30 | 5. Bleach silver           |      | 2  |
|    | 6. Rinse                   |      |    |
|    | 7. Fix                     |      | 4  |
|    | 8. Wash                    |      | 5  |
|    | 9. Dry (optional).         |      |    |
| 35 | 10. Color develop          |      | 10 |
|    | 11. Wash                   |      | 2  |
|    | 12. Harden                 |      | 1  |
|    | 13. Wash                   |      | 5  |

The above solutions had the following compositions:

|    |                                                   |   |      |
|----|---------------------------------------------------|---|------|
| 40 | Black-and-white developer:                        |   |      |
|    | 1-phenyl-3-pyrazolidone                           | g | 0.2  |
|    | Na <sub>2</sub> SO <sub>3</sub>                   | g | 1.0  |
|    | Na <sub>2</sub> CO <sub>3</sub> ·H <sub>2</sub> O | g | 20.0 |

45 H<sub>2</sub>O liter 1

|    |                               |       |      |
|----|-------------------------------|-------|------|
| 45 | Bleach:                       |       |      |
|    | Sodium potassium ferricyanide | g     | 15.0 |
|    | KBr                           | g     | 10.0 |
|    | H <sub>2</sub> O              | liter | 1    |

|    |                                                   |   |    |
|----|---------------------------------------------------|---|----|
| 50 | Color developer:                                  |   |    |
|    | 2-amino-5-diethylamino toluene·HCl                | g | 6  |
|    | Na <sub>2</sub> SO <sub>3</sub>                   | g | 2  |
|    | Na <sub>2</sub> CO <sub>3</sub> ·H <sub>2</sub> O | g | 20 |

H<sub>2</sub>O liter 1

55 In the above process a conventional acid hypo fixing solution was used for convenience at steps 3, 7 and 12. However, this solution need not contain hypo when used at steps 3 and 12, in which case it will be apparent that no silver halide will be removed from the emulsion layer at these steps.

As shown at stage 2 of the drawing, the result of the black-and-white development is to develop a silver image in area 12 of emulsion layer 11, and at the same time the hydroquinone derivative in the emulsion layer is oxidized to the quinonoid form in situ with the silver image. When a hardening and fixing solution has been employed at step 3, a large part of the silver halide is removed at this point in the process but as explained above, a silver halide solvent need not be present in this solution, in which case silver halide would not be removed from the element until step 7 has been carried out.

After bleaching and fixing the element, as in steps 5 and 7 above, the film appears substantially as shown at stage 3 of the drawing, the quinonoid image remaining in area 12 of the emulsion layer, residual unoxidized hydroquinone derivative in the remaining area of the emulsion layer and coupler compound remaining dispersed throughout the emulsion layer.

When color development has been carried out according to step 10 in the above process, it appears that the quinonoid image oxidizes the color developer in situ and the oxidized form of the color developer thus obtained then couples with the coupler compound in the emulsion layer to form a dye image in area 12 as shown in stage 4 of the drawings. The process as described yields a negative color reproduction of the subject but, as will be described hereinafter, may be adapted to the production of direct color reproductions.

The coupler compound used in the emulsion layer prepared as described above may be any of those well known in the art of color photography, such as the following:

1. 2 - (2',4'-di-t - amylophenoxyacetamido) - 4,6 - di-chloro-5-methyl phenol (Graham U. S. Serial No. 285,544, filed May 1, 1952) (blue-cyan)
2. 1 - hydroxy - 2[δ(2',4' - di - tert. - amylophenoxy) - n-butyl]naphthamide (U. S. 2,474,293) (grey-cyan)
3. 1 - (2',4',6' - trichlorophenyl) - 3 - [3" - (2'',4'' - di - tert. amylophenoxyacetamido) - benzamido] - 5 - pyrazolone (U. S. 2,600,788) (blue)
4. N - (p - benzoylacetaminobenzenesulfonyl) - N - (γ-phenylpropyl)-p-toluidine (U. S. 2,298,443) (yellow)
5. α - {3 - [α - (2,4 - di - tert. - amylophenoxy)acetamido]benzoyl}-2-methoxyacetanilide (McCrossen et al. U. S. Serial No. 476,159, filed December 20, 1954) (yellow)
6. 4,4' - p - methoxybenzylidene - bis - {1 - 2,4,6 - trichlorophenyl - 3 - [3" - (2'',4'' - di - tert. amylophenoxyacetamido)benzamido] - 5 - pyrazolone} (blue-grey)



A mixture of 33.6 parts of coupler 3 above, 3.4 parts of anisaldehyde and 125 volumes of ethanol was heated just below the boiling point for one hour and cooled overnight. The crystallized mixture was filtered and the product collected. The crude product was purified by crystallization from ethyl acetate to a melting point of 220°. 7. 1-phenyl-3-palmitoylamido-5-pyrazolone (blue).

One part of 1-phenyl-3-amino-5-pyrazolone was heated on the steam bath with 4 volumes of dioxane. To the hot mixture was added 1.6 parts of palmitoyl chloride and heating continued for 15 hours. The reaction mixture was cooled, filtered and the solid washed on the funnel with methanol until the washings were colorless. The product melting at 165-166° was collected. 8. 2 - cyanoacetylcoumarone - 5 - sulfon - N - (ω - phenylpropyl)-p-(tert.-amyl)aniline (orange-brown)



In a 3-l. three-necked flask, fitted with an efficient mechanical stirrer and a thermometer, is placed 1250 cc. (about 19 moles) of chlorosulfonic acid. The flask is cooled in an ice-salt freezing mixture to about -10° C., and to the cold acid, in small portions with vigorous stirring, is added 500 g. (2.7 moles) of the coupler 2-cyanoacetylcoumarone. The rate of addition should be such that the temperature does not rise above +5° C.; about 30 mins. is required. When all the coupler has been added, the mixture is stirred at 0° for 2 hrs. and then at room temperature overnight, or for about 15 hrs. Stirring is essential in part to prevent explosive foaming.

At the end of this time, the excess chlorosulfonic acid is decomposed by pouring the mixture with vigorous stirring onto 10 kg. of crushed ice. The decomposition is conveniently done in a 5-gal. crock, stirring and introducing the mixture simultaneously from two 1-l. dropping funnels. About 10 minutes is required for the decomposition. After being allowed to settle for a few minutes, the sulfonyl chloride is filtered off onto flannel, using two 12-inch Büchner funnels. The two cakes are combined, stirred with about 5 l. of ice water, and again filtered off on a large funnel. The cake is again broken up, and stirred this time with an ice cold solution of 500 g. of sodium acetate in 5 l. of water. The sulfonyl chloride is finally filtered off, washed on the funnel with about 5 l. of ice water, and sucked dry.

The cake, sucked as free as possible from water, is broken up and dissolved in 3 l. of 300 ethyl acetate. The ethyl acetate solution is dried over anhydrous magnesium sulfate and the ethyl acetate is distilled off under reduced pressure (40-50 mm. Hg), the distilling flask being heated in a water bath which has a temperature no higher than 60°. Toward the end of the concentration the temperature should be as low as 20°. The residue is stirred with 500 cc. of benzene, is filtered off, and washed on the filter with about 1 l. of ether. This washing removes a small amount of tarry impurity, which tends

to make the product sticky, and leaves the sulfonyl chloride as a light yellow powder which appears to be quite stable. The melting point of the pure material is 135-136°. The yield is about 250 g. (33%).

**2-cyanoacetylcoumarone-5-sulfon-N-(ω-phenylpropyl)-p-(t-amy)-aniline**

A mixture of 78.5 g. (.265 mole) of N-γ-phenylpropyl-p-t-amy-aniline, 24 g. (.29 mole) of anhydrous sodium acetate, and 75 g. (.264 mole) of 2-cyanoacetylcoumarone-5-sulfonyl chloride (added in the order given), in 350 cc. of glacial acetic acid, was stirred in a water bath at 50-55°. As the sulfonyl chloride went into solution sodium chloride started to precipitate. After running for 1 hour the reaction mixture set solid due to the crystallization of the product. The mixture was cooled in the ice box and filtered. After being sucked as dry as possible, the residue was washed on the filter with 100 cc. of methyl alcohol. The product was then slurried with 150 cc. of methyl alcohol, filtered, and rinsed with 50 cc. of methyl alcohol. This washing process was repeated using 200 cc. of ethyl ether and the residue rinsed with 200 cc. of ether till the filtrate was only faintly colored. After being sucked dry the product was washed in the same manner with water (300 cc. in all). It was then

air-dried, slurred with 150 cc. of ether, filtered and dried. Yield of cream-colored product, 72 g. (51.5%). M. P. 137-139°.

9. Di- $\beta$ -naphthoylmethane (blue-grey)



Sodamide was prepared from 4.6 parts of sodium and liquid ammonia. The ammonia was replaced by ether (250 volumes) and a solution of 20 parts of ethyl  $\beta$ -naphthoate and 17 parts of 2-acetonaphthone in 150 volumes of ether added. The mixture stood overnight, the solid was removed by filtration, suspended in water and acidified with acetic acid. The filtered product was recrystallized from acetic acid in pale yellow plates melting at 168-169°.

10. p-n-Amoxybenzoyl- $\beta$ -naphthoylmethane (green-grey)



In a 500-cc. three-necked flask are placed 17 g. (0.1 mole) of methyl  $\beta$ -naphthyl ketone and 90 g. (0.4 mole) of methyl p,n-amoxybenzoate. The flask is fitted with an eccentric type stirrer and a still head. The still head is connected through a water cooled condenser to a 500-cc. suction flask for removal of methanol during the reaction. The reaction flask is heated in an oil bath maintained at 165-175°, vigorous stirring is begun, and sodium methoxide is added in small increments. The reaction mixture turns dark immediately and methanol begins to distill. The additions which take about fifteen minutes are made as rapidly as evolution of methanol permits. The reaction mixture gradually thickens, and in about thirty minutes evolution of methanol ceases and the product sets to a solid mass. After heating fifteen minutes longer, the oil bath is removed and the flask chilled in running water.

The reaction mixture is stirred alternately with 100-cc. portions of water and benzene. This requires about 400 cc. of each to obtain solution of the whole mass. Ice is added to the emulsion which is then made acid to Congo red with dilute sulfuric acid. The benzene layer is next washed with three 200-cc. portions of 5% sodium bicarbonate, and with two 200-cc. portions of 5% sodium carbonate. The benzene layer is next washed with 200 cc. of 5% sodium hydroxide, and then shaken thoroughly with dilute sulfuric acid until the benzene layer is no longer cloudy. After another wash with dilute sodium bicarbonate, it is washed thoroughly with cold water until neutral. The benzene layer is then dried over calcium chloride, and concentrated in vacuo. The excess methyl p,n-amoxybenzoate is removed by careful distillation at low pressure. The recovered ester,

B. P. 1mm. = 132-135°

amounts to 45 g.

The residue is dissolved in 750 cc. of ethyl alcohol and treated with 1 g. of decolorizing charcoal. The solution is filtered hot through a steam heated fluted filter. The yield of product melting at 93-95° is 19.5 g. This is again crystallized from 500 cc. of alcohol giving 16 g. (44%) of light yellow flakes, M. P. 96-97°.

11. 1,3-diethylthiobarbituric acid (blue-grey) (J. A. C. S. 73, 5329 (1951))

In the above tabulation of coupler compounds, following the name of each of the compounds is given the approximate color of the dye image obtained when the given coupler is employed in the above process with the given color developing agent and given hydroquinone derivative in the emulsion layer.

It has been ascertained that when the first coupler compound of the above tabulation is used in the process, most of the dye in the resulting image is identical to that obtained in conventional color development processes in which color development takes place in the presence of the coupler and exposed silver halide. On the other hand, the dye image obtained when coupler No. 4 is used is a mixture of two yellow dyes in approximately equal amounts, it appearing that the quinonoid image obtained in this case during the black-and-white development step functions not only as an oxidizing agent for the color developing agent but also enters directly into the dye-forming reaction.

Dye image formation in the described process was most rapid and extensive when coupler compounds Nos. 1, 3, 4, 5 and 7 employed in the emulsion layer together with the mentioned hydroquinone derivative. These couplers are therefore preferred for use in my process.

Other hydroquinone derivatives which may be used in the emulsion layer prepared as described above include n-octadecylhydroquinone and 2-hexadecyl-6-methylhydroquinone. Dialkylhydroquinones, where both alkyl groups are larger than methyl, as, for example, 2,5-diethylhydroquinone, do not give dye images in this process.

The coupler solvent such as dibutyl phthalate employed for dispersing the hydroquinone derivative and coupler in the emulsion layer is not especially critical and can be selected from the substantially water-insoluble, low-molecular weight organic crystalloidal materials having a boiling point above about 175° C. disclosed, for example, in the Jelley and Vittum U. S. Patent 2,322,027 and other coupler solvents known in the art.

The developing agent used in the black-and-white developing solution of step 1 of the above process is fairly critical in that the developing agent should not be a color

35 developing agent such as a paraphenylenediamine compound but should have a high development activity and should be capable in the black-and-white development step of the process of leading to the oxidation of the hydroquinone derivative in the emulsion layer to the quinonoid form.

The p-aminophenols and N-alkyl o-aminophenols, such as p-aminophenol, 2-methyl-4-aminophenol, 2-methyl-4-diethylaminophenol, N-methyl-p-aminophenol, and o-methylaminophenol are very useful as well as the 3-pyrazolidone silver halide developing agents, a number of which are disclosed in the James et al.

45 U. S. Patent 2,688,549, granted September 7, 1954. In addition to 1-phenyl-3-pyrazolidone, 1-phenyl-4-methyl-3-pyrazolidone, 1-phenyl-4,4-dimethyl-3-pyrazolidone, and 1-p-tolyl-4,4-dimethyl-3-pyrazolidone are particularly

50 useful. 4-phenylcatechol was useful, and catechol was moderately effective. Hydroquinone and o-aminophenol were not useful in the process.

The color developing agents used in step 10 of the process are not especially critical and can be selected, for example, from the p-phenylenediamines known in the art, and can be expected to yield dye images of somewhat different color with a particular coupler compound.

55 My process can be adapted to the production of multi-color images by the incorporation of different coupler compounds in the emulsion layers of a multilayer film whose emulsions are sensitive to different regions of the spectrum. In this case the same hydroquinone derivative

60 or different hydroquinone derivative selected from those mentioned above as useful in the process, can be incorporated into the respective emulsion layers together with the given coupler compounds. A suitable film can have the usual red, green and blue-sensitive emulsion layers superimposed with a yellow filter between the green and blue-sensitive emulsion layers. In the emulsion layers

65 are incorporated coupler compounds such as those mentioned yielding subtractively colored dye images in the process. In case developing-out emulsions have been used in the emulsion layers, such multilayer elements are 70 adapted to the production of original color negatives, or

color negative transparencies may be printed thereon and color positives obtained by processing the film as described above.

Direct-positive color reproductions of a subject can be readily obtained using my process by employing in the sensitive elements a direct-positive silver halide emulsion such as the known internal latent image emulsions, in which case for the black-and-white development step of my process a developer may be used containing a suitable quantity of a hydrazine fogging agent. Emulsions and developers suitable for this purpose are described in the Haist et al. U. S. Patent 2,685,514, granted August 3, 1954. In the hydrazine-containing developers described in that patent, corresponding to the black-and-white developer of step 1 of my process described above, the p-aminophenol and 3-pyrazolidone developing agents mentioned above should be used, and if desired, these developing agents may be used in combination, for example, the combination of N-methyl-p-aminophenol sulfate together with 1-phenyl-3-pyrazolidone.

The process of my invention is applicable to the production of colored images in other kinds of emulsion layers such as mixed packet types of emulsion layers, in which case the hydroquinone derivative is incorporated along with the couplers in the packets.

What I claim is:

1. A photographic reproduction process which comprises exposing to a subject a silver halide emulsion layer containing a mixture of a coupler compound reactive with the oxidation product of a primary aromatic amino silver halide developing agent to form a dye and a hydroquinone derivative of the class consisting of n-octadecylhydroquinone, sec-octadecylhydroquinone and 2-hexadecyl-6-methylhydroquinone dispersed in the emulsion layer by means of a substantially water-insoluble, low 35

molecular weight, organic crystalloidal material having a boiling point above about 175°C., developing the exposed emulsion layer with an alkaline solution of a developing agent of the class consisting of p-aminophenol, N-alkyl-p-aminophenol, and 3-pyrazolidone silver halide developing agents thereby forming in the emulsion layer an image of silver and oxidized hydroquinone derivative, removing the silver image and residual silver halide from the emulsion layer, treating the remaining oxidized hydroquinone derivative image in the presence of the coupler compound with an alkaline solution of a p-phenylenediamine silver halide developing agent to form a dye image in the region of original silver image.

2. The process of claim 1 in which the coupler compound is 2-(2',4'-di-tert-amylphenoxyacetamido)-4,6-dichloro-5-methyl phenol.

3. The process of claim 1 in which the coupler compound is 1-(2',4',6'-trichlorophenyl)-3-[3''-(2''',4''-di-tert. amylphenoxyacetamido)-benzamido]-5-pyrazolone.

4. The process of claim 1 in which the coupler compound is 1-phenyl-3-palmitoylamido-5-pyrazolone.

5. The process of claim 1 in which the coupler compound is N-(p-benzoylacetaminobenzenesulfonyl)-N-( $\gamma$ -phenylpropyl)-p-toluidine.

25 6. The process of claim 1 in which the coupler compound is  $\alpha$ -(3-[ $\alpha$ -(2,4-di-tert-amylphenoxy)acetamido]-benzoyl)-2-methoxyacetanilide.

References Cited in the file of this patent

UNITED STATES PATENTS

|           |              |       |               |
|-----------|--------------|-------|---------------|
| 2,206,126 | Schinzel     | ----- | July 2, 1940  |
| 2,249,541 | Schinzel     | ----- | July 15, 1941 |
| 2,728,659 | Loria et al. | ----- | Dec. 27, 1955 |